



3



Exemplified compound No.

|              | $\text{R}_2$                                                                      | $\text{R}_4$                                                                      |
|--------------|-----------------------------------------------------------------------------------|-----------------------------------------------------------------------------------|
| [II]-16----- | $-\text{H}$                                                                       | $-\text{H}$                                                                       |
| [II]-17----- | $-\text{C}_2\text{H}_5$                                                           | $-\text{C}_2\text{H}_5$                                                           |
| [II]-18----- |  |  |
| [II]-19----- |  |  |
| [II]-20----- |  |  |
| [II]-21----- |  |  |
| [II]-22----- |  |  |
| [II]-23----- |  |  |
| [II]-24----- | $-\text{C}_{18}\text{H}_{35}$                                                     | $-\text{C}_{18}\text{H}_{35}$                                                     |

Examples of the compounds of the general Formula II

|  | $\text{X}'$ |  | $\text{SO}_2$                                                                        |  | $\text{X}$ | $\text{X}'$ |
|--|-------------|------------------------------------------------------------------------------------|--------------------------------------------------------------------------------------|------------------------------------------------------------------------------------|------------|-------------|
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |   |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |
|  |             |                                                                                    |  |                                                                                    |            |             |

sample was scanned by use of a microdensitometer having an open aperture of  $25\mu$ .)

TABLE 1

| Amount of compound (I) (g. per mole of $\text{AgX}$ ) | Amount of compound (II) (g. per mole of $\text{AgX}$ ) | Relative speed | Fog  | RMS |
|-------------------------------------------------------|--------------------------------------------------------|----------------|------|-----|
| [I]-4, 0.06 g.                                        |                                                        | 100            | 0.14 | 85  |
| [I]-4, 0.12 g.                                        |                                                        | 96             | 0.10 | 83  |
|                                                       | [III]-1, 1.4 g.                                        | 90             | 0.08 | 80  |
|                                                       | [III]-1, 2.8 g.                                        | 103            | 0.08 | 83  |
| [I]-4, 0.06 g.                                        | [III]-1, 1.4 g.                                        | 100            | 0.08 | 83  |
| [I]-4, 0.06 g.                                        | [III]-1, 2.8 g.                                        | 99             | 0.08 | 61  |
| [I]-9, 0.06 g.                                        | [III]-1, 1.4 g.                                        | 89             | 0.06 | 58  |
| [I]-13, 0.06 g.                                       | [III]-1, 1.4 g.                                        | 101            | 0.08 | 65  |
| [I]-18, 0.10 g.                                       | [III]-1, 1.4 g.                                        | 98             | 0.08 | 70  |
| [I]-4, 0.06 g.                                        | [III]-2, 1.4 g.                                        | 102            | 0.06 | 62  |
| [I]-4, 0.06 g.                                        | [III]-2, 1.4 g.                                        | 93             | 0.07 | 64  |
| [I]-4, 0.06 g.                                        | [III]-3, 1.4 g.                                        | 104            | 0.08 | 58  |
| [I]-4, 0.06 g.                                        | [III]-7, 1.4 g.                                        | 100            | 0.08 | 60  |
| [I]-4, 0.06 g.                                        | [III]-8, 1.4 g.                                        | 100            | 0.08 | 63  |
| [I]-4, 0.06 g.                                        | [III]-10, 1.4 g.                                       | 98             | 0.06 | 58  |
| [I]-4, 0.06 g.                                        | [III]-12, 1.4 g.                                       | 96             | 0.06 | 54  |

Coupler (4):





9

Formalin and 300 ml. of 5% saponin per mole of  $\text{AgX}$ , and coated on a triacetate film base to a dry film thickness of  $5\mu$ , followed by drying, to prepare a photographic film. The photographic film was exposed through an optical wedge to a light of regulated amount, developed at  $20^\circ \text{ C}$ . for 10 minutes by use of a color developer solution of the composition shown below, and then subjected to the same fixing and the like treatments as in Example 1.

#### Composition of color developing solution:

G.

|                                          |      |
|------------------------------------------|------|
| Anhydrous sodium sulfite                 | 2.0  |
| 4-amino-N,N-diethylaniline hydrochloride | 5.0  |
| Sodium carbonate (monohydrate)           | 50.0 |
| Potassium bromide                        | 1.0  |
| Water to make 1,000 ml.                  |      |

Water to make 1,000 ml.

TABLE 3

| Amount of compound (I)<br>(g. per mole<br>of AgX) | Amount of compound (II)<br>(g. per mole<br>of AgX) | Relative speed | Fog  | RMS |
|---------------------------------------------------|----------------------------------------------------|----------------|------|-----|
| [I]-9, 0.1 g.                                     | -----                                              | 100            | 0.10 | 92  |
| [I]-9, 0.1 g.                                     | [II]-6, 3 g.                                       | 96             | 0.06 | 88  |
| [I]-9, 0.1 g.                                     | [II]-6, 3 g.                                       | 98             | 0.08 | 90  |
| [I]-9, 0.1 g.                                     | {[II]-6, 2 g.<br>[II]-1, 1 g.}                     | 96             | 0.08 | 64  |
| [I]-9, 0.05 g.                                    | {[II]-6, 3 g.}                                     | 95             | 0.06 | 68  |
| [I]-2, 0.05 g.                                    | {[II]-6, 3 g.}                                     | 98             | 0.06 | 66  |

From Table 3, it is understood that marked improvement in graininess can be attained also in the case of a combination of two kinds of the compound (I) and one kind of the compound (II) or a combination of one kind of the compound (I) and two kinds of the compound (II).

**EXAMPLE 4**

A high speed, light-sensitive silver iodobromide photographic emulsion (containing 4.5 mole percent of AgI, and 160 g. of gelatin per mole of AgX) was subjected to second ripening, and then incorporated with 1.4 g./mole AgX of 5-methyl-7-hydroxyl-1,3,4-triazaindolizine and each of the two solutions (1) and (2) of the compositions shown below to prepare two green-sensitive emulsions.

10

### Composition of coupler dispersion:

|                             |    |       |
|-----------------------------|----|-------|
| Coupler (6)                 | g  | 82    |
| 2,5-di-(6-octylhydroquinone | g  | 3     |
| Tricresyl phosphate         | g  | 60    |
| Ethyl acetate               | g  | 250   |
| 5% alkanol B                | ml | 320   |
| 3% gelatin                  | ml | 2,000 |

Subsequently, each of the above-mentioned emulsions was mixed with the thus prepared coupler dispersion, charged with 120 ml. of 1% Formalin and 500 ml. of 5% saponin per mole of  $\text{AgX}$ , and coated on a triacetate film base to a dry film thickness of  $5\mu$ , followed by drying to prepare samples. These samples were subjected to the same treatments as in Example 1 to obtain the results as shown in Table 4.

TABLE 4

|           | Relative speed | Fog  | RMS |
|-----------|----------------|------|-----|
| Solution: |                |      |     |
| 1-----    | 100            | 0.10 | 88  |
| 2-----    | 100            | 0.07 | 64  |

25 As seen in Table 4, the sample according to the present invention is markedly improved in graininess without any loss in speed.

What we claim is:

1. A color photographic material containing a silver halide light-sensitive coupler-containing emulsion layer, at least one compound of the formula



40 wherein  $R_1$ ,  $R_2$  and  $R_3$  are individually hydrogen, lower

|                  | Solution |          |
|------------------|----------|----------|
|                  | 1, grams | 2, grams |
| Sensitizing dye: |          |          |
|                  | 0.2      | 0.2      |
| Compound (I)-5   | 0.06     |          |
| Compound (II)-4  |          | 2.00     |
| Methyl alcohol   | (i)      |          |

**1** 300 milliliters.

On the other hand, a coupler of the structure shown below was dispersed by means of a high speed rotary mixer together with such components as set forth below to form a coupler dispersion of the composition shown below, in which the amount of each component is per mole of  $\text{AgX}$ .

Coupler (6):



alkyl, alkenyl, aryl or aralkyl, and at least one compound of the formula



wherein  $R_4$  is hydrogen, lower alkyl, or aralkyl, and  $X$  and  $X'$  are individually hydrogen, alkyl, alkoxy or halogen.

2. The photographic material according to claim 1, wherein the compound of the Formula I and the compound of the Formula II individually are incorporated into two separate and adjacent layers of said material.

75 3. The photographic material according to claim 1,

**11**

wherein the compound of the Formula I and the compound of the Formula II are incorporated into the same layer of said material.

4. The photographic material according to claim 1, wherein the alkenyl group is



or

**12**

## References Cited

## UNITED STATES PATENTS

|             |        |                        |        |
|-------------|--------|------------------------|--------|
| 3,295,976   | 1/1967 | Abbott et al. -----    | 96-109 |
| 3,311,474   | 3/1967 | Willems et al. -----   | 96-109 |
| 5 3,554,756 | 1/1971 | Terashima et al. ----- | 96-100 |

J. TRAVIS BROWN, Primary Examiner

U.S. Cl. X.R.

10 96-55, 74, 109